

1

3,140,197

## FINISHED TEXTILE AND METHOD OF PRODUCING SAME

Georg Heberlein, Fritz Munzel, and Werner Kunz, Wattwil, Switzerland, assignors to Heberlein & Co. AG., Wattwil, Switzerland, a corporation of Switzerland  
No. Drawing. Filed Mar. 31, 1960, Ser. No. 62,068  
Claims priority, application Switzerland Apr. 1, 1959  
8 Claims. (Cl. 117—93.31)

This invention relates to an improved method of finishing textiles to impart dimensional stability and crease-resistance thereto. It is particularly directed to a method of finishing a textile formed from natural or regenerated cellulose, and is especially adapted for imparting "wash and wear" properties to cellulosic textile materials. This invention is also directed to a finished natural or regenerated cellulose textile product characterized by a high resistance to creasing, excellent dimensional stability by a higher abrasion resistance than the unfinished textile.

The term "textile" as employed herein shall be understood to include textile materials of all kinds, including fibers, yarns, threads, and woven as well as non-woven fabrics and knitted goods.

It is known that in order to improve the crease-resistant properties of natural or regenerated cellulose fabrics, for example, cotton or rayon or mixed cotton and rayon goods, the fabric is impregnated with one or more well known condensable substances, for example, a synthetic resin precondensate, which is dispersed or dissolved in a carrier which also contains a condensation catalyst. Following impregnation, the excess resin is squeezed out and the impregnated fabric is then subjected to elevated temperatures, above 100° C., for a period of time sufficient to condense the resin. This technique is "conventional" in the art and is so referred to hereinafter. Cellulosic textiles finished in the conventional manner with the aid of elevated temperature are generally speaking substantially less durable than the unfinished or starting fabric. For example, the conventional finishing method imparts acceptable crease-resistance, but at the expense of a marked reduction in the fiber strength of the textile product, as evidenced by either an appreciably reduced tensile strength or resistance to abrasion or both.

It is an object of the present invention to provide a method for finishing cellulosic textile materials which does not employ elevated temperature to effect condensation of the condensable finishing substance on the textile. It is a further object to produce a dimensionally stable cellulosic textile having excellent crease-resistant properties without adversely affecting the tensile strength or abrasion resistance of the goods. It is another object of the present invention to provide a novel resin-finished textile of superior tensile strength and abrasion resistance than the conventional thermally condensed resin-finished textile.

In accordance with the method of the present invention it has now been found that cellulosic textiles, especially flat shaped fabrics, can be finished in an improved manner, without resort to the elevated temperatures of the conventional process, by first treating the textile with a condensable substance and then subjecting the treated textile to the influence of ionizing radiation, more particularly to electromagnetic ionizing radiation, namely

2

gamma radiation or X-rays, whereby the condensable substance is condensed on the textile.

The terms "condensable substance" and "resin precondensate" are employed interchangeably herein and are to be understood as meaning a substance which can be condensed with itself and with cellulose; these terms may also refer to a mixture of two or more substances which may intercondense. These "condensable substances" are those customarily employed in the crease-proof finishing of cellulosic textiles, and are well known cross-linking or resin-forming substances, for example, methylol ureas, methylol amines, precondensates of formaldehyde with phenol and phenol derivatives, ketone-aldehyde precondensates, aziridinyl compounds, diglycide ethers. 15 Other suitable resin-forming substances are N-substituted urea formaldehyde resin compositions such as ethylene urea, dioxy ethylene urea or N,N'-bis (methoxy-methyl) 20 uron and tetrahydro-1,3-bis (methoxymethyl)-5-methyl-2(1)-s-triazine as described in United States Patent No. 2,373,135. Mixtures of two or more condensable substances may be employed if desired, as pointed out hereinafter by way of example.

In many instances the present method permits condensation of the resin-precondensate without resort to a catalyst, which is highly desirable since the cross-linking or condensing catalysts employed in the conventional process (e.g., metal halides, zinc nitrate, boron trifluoride, etc.) are acidic and adversely affect the cellulose. Whenever a catalyst is employed it is of course necessary to 25 thoroughly wash the textile in order to prevent damage to the cellulosic fibers. In some instances of the present method, after-washing may thus be eliminated.

The condensable substance is applied to the cellulosic textile in the form of a solution or dispersion in water or 30 an organic solvent, depending upon its nature and solubility. Impregnation of the textile is carried out in substantially the same manner as in the conventional finishing process, although with the present invention the squeezed-out textile may or may not be dried prior to 40 irradiation, if desired.

The total irradiation dose to which the impregnated fabric is subjected will depend upon the condensable substance with which the textile has been impregnated, with due care being taken to avoid any appreciable damage 45 to the cellulose molecule. The time required to effect condensation will of course depend upon the energy of the radiation source, and accordingly we specify herein a total dose in roentgen units (r.) to which the impregnated textile is subjected. We have found that a dose of 50 at least  $10^3$  r. is required, and that the dose should not exceed about  $10^7$  r. If the textile is subjected to more than about  $10^7$  r. serious degradation of the cellulose molecular structure results. Excellent results are obtained by irradiating the impregnated textile with gamma or 55 X-rays to a total dose of between about  $0.5 \times 10^6$  and about  $3 \times 10^6$  r. The irradiation may be carried out at room temperature, for example between about 15 and 25° C.

The most convenient sources of gamma-rays, the preferred electromagnetic ionizing radiation, are  $\text{Co}^{60}$ , "burnt" uranium slugs, fission products of  $\text{U}^{235}$ , separated isotopes, such as  $\text{Cs}^{137}$ , etc.

The method of the present invention employing electromagnetic ionizing radiation is not to be confused with

prior attempts by others to treat textiles which have been impregnated with condensable substances with high energy electron beams (beta particles) produced by high voltage accelerating apparatus, for example, to effect condensation. As a result of such a treatment with particles of an energy above about 1 mev. the cellulosic fibers which make up the textile are subjected to excessive degradation. In accordance with the present invention, on the other hand, the dose of ionizing radiation is relatively much smaller, so small that any decrease in strength or stability of the cellulosic fibers due to irradiation is negligible. As a practical matter, in nearly every instance the product of this invention exhibits a higher tensile strength and resistance to abrasion than the starting or unfinished textile. The reasons for this enhancement of the finished textile are not yet fully apparent, but may be in connection with cross-linking between resin and cellulose, although we do not wish to be bound by that hypothesis. While this invention is applicable to the treatment of cellulosic textiles of all kinds to impart crease-resistance and dimensional stability thereto, its electromagnetic ionizing radiation-induced condensation is also suitable for producing permanent effects in or on a textile fabric, for example, embossing effects such as goffering, ribbing, schreiner or moire effects, as well as calendering effects, produced with or without friction.

The present method is also eminently well suited for imparting a high degree of crease-resistance to parchmentized or transparentized natural or regenerated cellulose fabrics. As is known, a cellulosic fabric upon treatment with concentrated sulphuric acid becomes stiff and transparent. Similar effects can be obtained by treating the fabric with a cuprammonium solution or a sodium zincatecellulose solution. However, attempts to render such transparentized fabrics crease-resistant by condensing a resin precondensate thereon at temperatures of 100° C. and above in the conventional manner have resulted in a commercially untenable reduction in the strength of the fibres of the fabric which are already somewhat brittle by reason of the transparency treatment. If the transparentized fabrics are subjected to electromagnetic ionizing radiation in accordance with the present invention the resin precondensate is effectively condensed, and the resulting fabric product exhibits good crease resistance without any noticeable reduction in the strength of the fibers, that is, without any reduction in the tensile strength or abrasion resistance of the transparentized goods.

The invention is described in further detail in the following non-limiting examples which illustrate practical applications of the method, and describe certain characteristics of the novel finished textile products.

#### Example 1

A cotton imitation poplin with 36/19 threads per  $\frac{1}{4}$  French inch and English yarn numbers 40/30 in the warp and filling was singed, desized and bleached. It was then impregnated with a solution of 100 g. of dimethylol urea dissolved in one liter of water to which there was also added 11 g. of zinc nitrate catalyst. The fabric was then squeezed out and dried for twenty minutes at 60–70° C. It was then subjected to gamma radiation at 20° C. to a total dose of about  $1 \times 10^6$  r.  $\text{Co}^{60}$  having a radiation intensity of  $3.8 \times 10^5$  r. per hour was employed as the source of gamma rays. Following irradiation the fabric was washed and dried. The finished cotton cloth had a pleasantly soft hand.

The crease resistance of the finished fabric was determined by measuring crease angles as follows: Strips of the fabric 3 x 5 cm. conditioned for twenty-four hours at 21° C. and 65% relative humidity. They were thereupon folded in the warp or filling direction, respectively, and placed under a 1 kg. weight for one hour. Upon removal of the weight, the fabric samples were left unweighted for fifteen minutes and the crease angle thereupon measured.

5 The tensile strength of the fabric was measured with a Schopper pendulum apparatus on strips 2.5 cm. wide. Abrasion resistance was measured with a standard testing apparatus containing a disc covered with a standardized wool cloth which was rotated on the surface of the fabric until the fabric failed, and the number of revolutions to failure was noted.

10 The warp and filling crease angles, tensile strength and abrasion strength of the unfinished and finished fabric along with values for the same fabric which was finished in the conventional manner with the same condensable substance, but with condensation being effected by subjecting the fabric to a temperature of 140° C. for five minutes, are reported below

|                      | Unfinished | Finished | Conven-tion-ally Finished |
|----------------------|------------|----------|---------------------------|
| Warp angle (deg.)    | 44         | 107      | 113                       |
| Filling angle (deg.) | 40         | 100      | 114                       |
| Tensile (kg.)        | 23         | 30       | 14.5                      |
| Abrasion (revs.)     | 15,000     | 43,000   | 3,170                     |

#### Example 2

A desized mercerized bleached cotton poplin fabric was impregnated with a 10% aqueous solution of a triazone derivative of the following formula:



35 which contained no catalyst. The impregnated fabric was dried for ten minutes at 60–70° C. and then subjected to the action of gamma radiation at 20° C. to a total dose of  $2 \times 10^6$  r. Fission products of  $\text{U}^{235}$  having an intensity of  $8 \times 10^6$  r. per hour were employed as the source. Following the irradiation-induced condensation of the triazone derivative, it was unnecessary to wash the fabric since no catalyst was employed. The finished fabric had a pleasantly soft hand.

40 The crease angles, tensile and abrasion strengths of the unfinished and finished fabric were as follows:

|                      | Unfinished | Finished |
|----------------------|------------|----------|
| Warp angle (deg.)    | 45         | 81       |
| Filling angle (deg.) | 56         | 79       |
| Tensile (kg.)        | 22.8       | 21.7     |
| Abrasion (revs.)     | 15,800     | 16,100   |

#### Example 3

A cotton longcloth which had been pre-treated in the customary manner was impregnated with a 15% aqueous solution of aziridinyl phosphonium oxide of the following formula:



60 The solution also contained 15% of 65% boron trifluoride dihydrate (calculated on the aziridinyl compound) as catalyst, as well as 7.5% of 10% octadecylethyleneurea emulsion (calculated on the aziridinyl compound) as a plasticizer. Following impregnation the fabric was dried for ten minutes at 60–70° C., and then subjected to the source of gamma radiation of Example 2 at 20° C. to a total dose of about  $1 \times 10^6$  r. The finished fabric had a pleasantly soft hand and was substantially flame-proof.

Crease angles and values for tensile and abrasion strengths of the unfinished and finished fabric, as well as for a conventionally finished fabric (condensation having been effected by subjecting the impregnated cloth to temperature of 140° C. for a period of five minutes) were as follows:

|                      | Unfinished | Finished | Conventionally Finished |
|----------------------|------------|----------|-------------------------|
| Warp angle (deg.)    | 49         | 105      | 89                      |
| Filling angle (deg.) | 59         | 101      | 95                      |
| Tensile (kg.)        | 20         | 21       | 15.2                    |
| Abrasion (revs.)     | 10,000     | 15,500   | 12,800                  |

*Example 4*

A partially water soluble diepoxyde compound is prepared by interaction of glycerol monochlorhydrin and epichlorhydrin. An emulsion is formed by mixing 100 grams of this diepoxyde compound, 100 grams of a 5% polyvinyl alcohol solution and 20 grams of a 20% dispersion of a polyethylene softener. To this emulsion are added 12.5 grams of a 40% solution of zinc boronfluoride; water is then added with intense stirring to make a liter of emulsion.

Cotton poplin was impregnated with this dispersion, and then subjected, without preliminary drying, to Co<sup>60</sup> to a total dose of gamma radiation equal to about  $1 \times 10^6$  r. Irradiation was carried out at 23° C. Following irradiation the fabric was washed and dried. The finished fabric was found to be absolutely resistant to chlorine washing, and the quantity of resin on the fabric was not affected by repeated immersions in boiling water.

Crease angles and tensile and abrasion strengths of the unfinished and finished fabric, as well as those for the same fabric conventionally finished with the same resins which were condensed by subjecting the impregnated fabric to a temperature of 140° C. for five minutes, were as follows:

|                      | Unfinished | Finished | Conventionally Finished |
|----------------------|------------|----------|-------------------------|
| Warp angle (deg.)    | 48         | 95       | 70                      |
| Filling angle (deg.) | 45         | 92       | 83                      |
| Tensile (kg.)        | 26         | 43       | 15.5                    |
| Abrasion (revs.)     | 12,000     | 17,000   | 8,990                   |

The fabric finished in accordance with the present invention was then washed six times, each for a period of thirty minutes at 95° C., with an aqueous solution containing 5 g. of soap and 2 g. of soda per liter, and then dried. The crease angles and tensile and abrasion strengths following washing were as follows:

**FINISHED FABRIC AFTER WASHING**

|                      |        |
|----------------------|--------|
| Warp angle (deg.)    | 91     |
| Filling angle (deg.) | 95     |
| Tensile (kg.)        | 42     |
| Abrasion (revs.)     | 16,000 |

*Example 5*

A dispersion was prepared which contained 100 g. of a 5% polyvinyl alcohol solution, 25 g. of a nonionic plasticizer, 75 g. of the diepoxyde of Example 4, 60 g. of a 50% solution of dimethylolethyleneurea and 13 g. of a 40% zinc boronfluoride solution in 750 g. of water. A fabric containing warp and filling yarns of 70% cotton-30% spun rayon, which had been pretreated in the customary manner and mercerized was impregnated with the aforementioned dispersion and squeezed out to 85%. Thereupon, the fabric was dried for thirty minutes at 50° C. and irradiated at 18° C. with Co<sup>60</sup> to a total gamma radiation dose of about  $1.3 \times 10^6$  r. Upon washing with 5 g. per liter soap at 60° C. in a washing machine fol-

lowed by drying the dimensions of the finished fabric did not change for practical purposes.

The crease angles and tensile and abrasion strengths of the unfinished and finished fabric were as follows:

|                      | Unfinished | Finished |
|----------------------|------------|----------|
| Warp angle (deg.)    | 47         | 105      |
| Filling angle (deg.) | 40         | 95       |
| Tensile (kg.)        | 13         | 13       |
| Abrasion (revs.)     | 12,000     | 16,000   |

*Example 6*

Spun rayon gabardine was impregnated with an aqueous solution of a urea-formaldehyde precondensate containing 10% MgCl<sub>2</sub>·6H<sub>2</sub>O and an equal weight of a silicone emulsion (both magnesium chloride and silicone emulsion being calculated on the weight of urea-formaldehyde pre-condensate). The fabric was then squeezed out to 90%, and without further drying subjected at 20° C. to Co<sup>60</sup> to a total gamma radiation dose of about  $0.8 \times 10^6$  r. Following irradiation the fabric was finally dried under tension. It had a pleasantly soft hand.

The crease angle and tensile and abrasion strengths of the finished and unfinished fabric were as follows:

|                      | Unfinished | Finished |
|----------------------|------------|----------|
| Warp angle (deg.)    | 45         | 110      |
| Filling angle (deg.) | 43         | 110      |
| Tensile (kg.)        | 23         | 34       |
| Abrasion (revs.)     | 14,000     | 19,000   |

The textile materials of Examples 1-6 are considered light to medium weight fabrics, and in each instance the finished product still retained a pleasantly soft hand.

While the treating conditions set forth in Examples 1-6 are not offered as optimum, but simply as illustrative of the present method, nevertheless, examination of the crease angles, tensile and abrasion strengths reported for each of the six products clearly shows the markedly improved crease-proof properties of the finished goods as well as the marked improvement in resistance to abrasion as compared with the unfinished material. Furthermore, in nearly every instance the tensile strength of the unfinished goods is very significantly increased. Tensile strength is never substantially reduced.

In Examples 1, 3 and 4 comparisons of the present product with that produced by the conventional method are given. Tensile and abrasion strengths of the present product are materially higher than for the conventional product, with substantially the same or a greater improvement in the crease angles.

*Example 7*

A bleached mercerized cotton-make yarn of English yarn number 60/2 was impregnated with an aqueous solution containing 70 g. of dimethylolethyleneurea and 10 g. of zinc nitrate per liter, dried at 60° C. and then subjected at 20° C. to gamma radiation from Co<sup>60</sup> to a total dose of about  $1 \times 10^6$  r. The finished yarn is eminently well suited for embroidery and has less tendency to shrink than the unfinished yarn or yarn finished by the conventional method.

*Example 8*

A cotton muslin of 29/19 threads per 1/4 French inch and English yarn number 80/102 in the warp and filling was mercerized and bleached in the usual manner. It was then treated with 50.7° Bé. sulfuric acid at 15° C. for seven seconds, washed with water, after-mercerized with 30° Bé. caustic soda for fifteen seconds, then washed neutral in cold water and dried under tension. This pre-treatment produced a transparentized fabric, which was then impregnated with a solution of 110 g. of dimethylolethyleneurea dissolved in one liter of water to which

had been added 11 g. of zinc nitrate. The transparentized fabric was then squeezed out and dried for twenty minutes at 60-70° C. The thus transparentized, impregnated dried goods were then subjected at 20° C. to gamma radiation from a Co<sup>60</sup> source having an intensity of  $3.8 \times 10^5$  r. per hour to a total dose of about  $1 \times 10^6$  r.

After irradiation the fabric was washed and dried under tension. The crease angles of the transparentized unfinished fabric and the finished fabric were as follows:

|                | Unfinished | Finished |
|----------------|------------|----------|
| Crease angle:  |            |          |
| Warp (deg.)    | 30         | 66       |
| Filling (deg.) | 20         | 62       |

*Example 9*

The mercerized bleached cotton fabric of Example 8 was parchmentized by treatment with 52.5° Bé. sulfuric acid at 15° C. for sixteen seconds, and then after-mercerized with 30° Bé. caustic soda for fifteen seconds. The resulting fabric was washed to neutral with cold water, dried under tension and then impregnated with a 10% aqueous solution of 1-carbonyl-2,5-dimethoxy-4-ethyl-triazin-2,4,6 and dried at 60-70° C. The thus impregnated parchmentized fabric was then irradiated with Co<sup>60</sup> at 20° C. to a total gamma radiation dose of about  $2 \times 10^6$  r. The crease angles of the parchmentized unfinished starting material and the resin finished fabric were as follows:

|                | Unfinished | Finished |
|----------------|------------|----------|
| Crease angle:  |            |          |
| Warp (deg.)    | 14         | 62       |
| Filling (deg.) | 11         | 71       |

*Example 10*

The mercerized bleached cotton fabric of Example 8 was treated for ten seconds with a cuprammonium solution containing 18 g. copper, 150 g. ammonia and 10 g. caustic soda per liter, and subsequently freed of copper by treatment with dilute sulfuric acid and then thoroughly rinsed with water. It was after-mercerized with 30° Bé. caustic soda for fifteen seconds, washed to neutral with water and dried under tension. The thus pretreated fabric was then impregnated with the aqueous aziridinyl phosphonium oxide solution of Example 3, and then dried for ten minutes at 60-70° C. It was thereupon subjected to Co<sup>60</sup> at 20° C. to a total gamma radiation dose of about  $1 \times 10^6$  r.

The crease angles of the transparentized unfinished material and that of the finished fabric were as follows:

|                | Unfinished | Finished |
|----------------|------------|----------|
| Crease angle:  |            |          |
| Warp (deg.)    | 10         | 90       |
| Filling (deg.) | 10         | 90       |

*Example 11*

The mercerized bleached cotton fabric of Example 8 was transparentized by treatment with an aqueous sodium zincate-cellulose solution containing 50 g. cellulose, 20 g. zinc oxide, and 75 g. caustic soda per liter, after which it was squeezed off, immersed in dilute sulfuric acid, washed with water and after-mercerized with 30° Bé. sodium hydroxide and dried under tension. The transparentized fabric was impregnated with a solution containing per liter:

Urea-formaldehyde precondensate (45%) \_\_\_\_cc\_\_\_\_ 300  
Magnesium chloride \_\_\_\_\_g\_\_\_\_ 13  
Silicone emulsion \_\_\_\_\_g\_\_\_\_ 13

and then squeezed out and without further drying sub- 75

jected at 20° C. to gamma radiation to a total dose of about  $1 \times 10^6$  r., after which it was dried under tension. The crease angles of the transparentized unfinished material and that of the finished fabric were as follows:

|                | Unfinished | Finished |
|----------------|------------|----------|
| Crease angle:  |            |          |
| Warp (deg.)    | 24         | 45       |
| Filling (deg.) | 20         | 45       |

*Example 12*

A spun rayon muslin with 23/21 threads per  $\frac{1}{4}$  French inch and English yarn number 60/70 in the warp and filling was scoured in the usual manner and dried under tension. It was then treated with 47° Bé. sulfuric acid at 10° C. for ten seconds, washed with water, after-mercerized with 30° Bé. caustic potash for five seconds, washed to neutral with hot water and then dried under tension. The so pretreated fabric was then impregnated with the urea-formaldehyde precondensate solution of Example 11, squeezed out, dried under tension and subjected at 20° C. to gamma radiation to a total dose of about  $1 \times 10^6$  r. This finishing technique resulted in a substantial improvement in the crease resistance of the transparentized fabric.

As a result of the parchmentizing or transparentizing techniques of Examples 8-12 the tensile strength and elongation at break of the starting fabric are as a rule slightly reduced. However, the irradiation-induced condensation of the condensable substance in accordance with the method of the present invention did not, for all practical purposes, further reduce the tensile or abrasion strength of the transparentized or parchmentized fabric.

As respects tensile and abrasion strengths, the finished fabric products of the Examples 8-12 were substantially the same as those of the starting transparentized material, although the crease resistant properties of the transparentized fabric were very markedly improved, as shown. In each example there was improvement in excess of 150% in warp and filling directions.

In each of the above fabric examples the dimensions of the goods following washing did not change for all practical purposes, and the fabrics can be said to exhibit excellent dimensional stability.

While this invention is concerned with an improved finishing method for cellulosic textiles and the improved finished cellulosic textile product it is not to be inferred from the above description or the appended claims that the textile being finished or the finished product consist entirely of natural or regenerated cellulose or a mixture of these cellulosic materials. Cellulosic materials must constitute a major portion of the textile product or textile being finished, but textiles containing in addition a small quantity of non-cellulosic fibers or filaments are also within the scope of this invention.

We claim:

1. A method of finishing a cellulosic textile, which comprises impregnating the textile with a condensable crease-resistance imparting finishing substance dispersed in a fluid carrier and then subjecting the impregnated textile to high energy ionizing radiation to a total radiation dose in the range between about  $10^3$  and about  $10^7$  r. to condense the condensable substance on the textile without substantially reducing the strength of the textile.

2. A method as set forth in claim 1 wherein the impregnated textile is irradiated at between about 15 and 25° C.

3. A method as set forth in claim 1, wherein the total radiation dose is between about  $0.5 \times 10^6$  and about  $3 \times 10^6$  r.

4. A method as set forth in claim 1 wherein the impregnated textile is irradiated in squeezed out but moist condition.

5. A method as set forth in claim 1 wherein the impregnated textile is dried prior to irradiation.

6. A crease resistant, cellulosic textile finished by the process of claim 1.

7. A method for imparting wash and wear characteristics to a cellulosic textile material, which comprises impregnating the textile with a wash and wear resin precondensate in a fluid carrier and then subjecting the impregnated textile to high energy ionizing radiation to a total radiation dose in the range of about  $0.5 \times 10^6$  to about  $3 \times 10^6$  r. to condense the resin precondensate without substantially impairing the strength of the textile.

8. A transparentized crease resistant, cellulosic textile fabric finished by the process of claim 7.

References Cited in the file of this patent

UNITED STATES PATENTS

|    |           |                |       |               |
|----|-----------|----------------|-------|---------------|
| 15 | 1,818,073 | Long           | ----- | Aug. 11, 1931 |
|    | 1,985,124 | Weiss          | ----- | Dec. 18, 1934 |
| 5  | 2,373,135 | Maxwell        | ----- | Apr. 10, 1945 |
|    | 2,545,540 | Dalton         | ----- | Mar. 20, 1951 |
|    | 2,670,483 | Brophy         | ----- | Mar. 2, 1954  |
| 10 | 2,833,674 | Hurwitz        | ----- | May 6, 1958   |
|    | 2,921,006 | Schmitz et al. | ----- | Jan. 12, 1960 |
|    | 2,950,553 | Hurwitz        | ----- | Aug. 30, 1960 |
|    | 2,998,329 | Sovish et al.  | ----- | Aug. 29, 1961 |

FOREIGN PATENTS

|    |                  |        |       |               |
|----|------------------|--------|-------|---------------|
| 15 | 66,034/1,070,401 | France | ----- | Apr. 24, 1956 |
|----|------------------|--------|-------|---------------|